

## UNITED STATES PATENT OFFICE

CARLETON ELLIS, OF MONTCLAIR, NEW JERSEY, ASSIGNOR TO ELLIS-FOSTER COMPANY, A CORPORATION OF NEW JERSEY

## PAPER PRODUCT

No Drawing.

Application filed June 18, 1928. Serial No. 286,485.

This invention relates to a paper product containing oxidized paraffin wax, and the like, and to containers and container closures made from such paper material.

5 This application is derived in large measure from my copending application Serial No. 107,461, filed November 15, 1928.

Oxidized paraffin may be prepared by blowing a current of air or oxygen, or other oxygen-containing gas through the molten material for a period of several hours, the temperature usually ranging from 160-200° C. Oxygen goes into combination and to a certain extent fatty acids are formed together with various other oxygenated products. For the purposes of the present invention I prefer to carry the treatment only to a stage of incipient oxidation, the blown material containing a minimum of fatty acids, and the like. Preferably in the case of wax the oxidation is merely sufficient to somewhat reduce the greasiness of the wax and permit it to disperse more readily in an aqueous medium. By blowing wax for several hours at a temperature of 160° C. but stopping the operation before deep-seated changes take place, a product which has been thus subjected to incipient oxidation results which is desirably employed in carrying out the purposes 20 of the present invention.

The blown wax in a stage of incipient oxidation is mixed with pulp, preferably in the beater engine, or any other suitable stage in advance of actual formation into a sheet. 35 Two or three per cent by weight of the blown wax, based on the paper material, may be introduced advantageously in this manner. Wax in this proportion, or even in lesser relative amount creates a desirable waterproofing effect.

The paper stock may be ordinary sulphite pulp, or it may be derived from pulp produced by other processes of treating wood, or mixtures of pulps obtained from different 45 processes. In some cases ground wood, or

mixtures of ground wood with sulphite pulp or other pulp may be employed. The invention is not restricted to paper made from various forms of wood pulp, but may include stock made, for example, from jute and 50 analogous fibres.

Difficulty has arisen in the past in the endeavor to use paraffin wax in paper pulp due to clogging of the felts and screens with wax. In the present invention it is proposed to 55 oxidize the wax to a stage sufficient to render its dispersion in water to be very thorough and permit of more effective occlusion of the dispersed blown wax by the wet paper pulp.

The exact degree of waterproofing or water 60 resistance created depends, however, on the requirements of service conditions, and in some cases a waterproofing effect of comparatively slight degree may be all that is required, while in other cases, a much more 65 substantial degree of water resistance is needed. The blown wax therefore, should be used in such proportion as meets the specific requirements in hand.

The blown wax may be used in conjunction 70 with rosin size, or other paper sizing agent. Alum, aluminum hydrate and various other coagulating agents for size may be used as required.

Instead of using the harder and more expensive grades of paraffin wax, it is possible to use in the present invention various cheaper grades of wax including scale wax or wax which has been softened with various oils. Thus in some instances I prefer to employ 80 the emulsion or dispersion of a mixture of wax and a good grade of petroleum oil, such mixture having been air-blown to at least a state of incipient oxidation. For a very high grade paper I may employ a blown mixture 85 of wax and one of the so-called medicinal petroleum oils, of which products oil such as "Nujol" or "Markol" are typical. For lower grades of paper, especially when color is not important, various petroleum oils admixed 90

with wax may be blown to yield an oxidized product which when dispersed in an aqueous medium may be readily incorporated in the wet paper pulp.

5 While I have specified wax in particular, I may include mixtures of paraffin wax in the oxidized form with other waxes such as carnauba, candelilla, Montan, ceresin, and the like. It is also possible to make a mixture 10 of waxes and blow these to oxidize them simultaneously and prepare the dispersion from this composite oxidized waxy material. Thus paraffin wax with 5 to 10 per cent of montan wax may be blown with air at a temperature of say, 170° C. for five hours. In 15 like manner blown mixtures of paraffin wax, petroleum oil and montan wax or other wax of a character different from paraffin wax may be blown and thus oxidized.

20 The dispersion of the oxidized material may be made in various ways, preferably with the aid of one or more emulsifying agents such as soap, alkali, starch, bentonite, silicate of soda, and the like. Thus a few per cent 25 of stearic or oleic acid may be melted with the oxidized paraffin and this composition emulsified with a hot, dilute, aqueous solution of caustic soda or ammonia. The ammonia composition is preferable in some cases because 30 any free ammonia may be removed very readily. Or, silicate of soda may be incorporated with the oxidized material and sufficient water to produce a creamy dispersion, and the mixture passed through an emulsifying apparatus such as a colloid mill. Using 35 a colloid mill, the amount of dispersing agent may be quite small. This is advantageous when ordinary soaps are employed because these tend to produce foaming in the beater 40 and therefore the proportion of these should be kept at a minimum. Less than 1 per cent of potassium or sodium oleate may be employed to make a satisfactory dispersion of oxidized paraffin wax in water. The dispersion 45 may contain about 50 per cent of wax and yet be readily handled.

As indicated above, the oxidized paraffin emulsion may be added to the beater engine which advantageously may be done at the 50 time the paper stock is charged thereinto. After thorough mixing in the usual manner in the beater a quantity of rosin size or any other desired sizing agent may be added and such size set in the usual manner with alum or 55 with any other setting agent. The addition of rosin size or similar sizing agent is, however, not necessary in making various forms of paper, it being proposed to produce paper without a sizing agent of a resinous character, if so desired, employing solely the oxidized material aforesaid to create adequate water resistance for the purpose in hand.

60 A paper pulp which contains a substantial proportion of hydrocellulose is advantageous 65 in assisting in the fixation of the oxidized

wax. The hydrocellulose may be added to the pulp or formed in it in any suitable manner.

The invention may be illustrated by the following:

A mixture of equal parts by weight of sulphite pulp and ground wood is agitated in water in the beater with a dispersion of oxidized paraffin wax sufficient to introduce about 4 per cent of wax into the finished 70 paper. The dispersion of the blown wax is made by violent agitation of equal volumes of the wax and a 1 per cent solution of sodium or potassium oleate. Agitation in the beater is continued until hydrocellulose is 75 formed to a considerable extent. After thorough admixture in this manner rosin size is added sufficient to introduce 1 or 2 per cent of rosin or resinate and this rosin size is set by alum, either already present in the beater, 80 or added after the rosin size has been incorporated. The proportion of alum introduced is sufficient to react both with the alkali of the rosin size and with that of the sodium or potassium oleate employed in dispersing the 85 blown wax.

The pulp so treated is formed into a sheet of paper which may be of single layer construction or may be built up in the paper machine in several layers to form a board. 95 Whether made in single sheet or single layer form, or built up in a plurality of layers, I include under the designation paper these and other varied forms of sheeted paper pulp.

The sheet is then calendered, preferably 100 hot, and the particles of oxidized wax, oxidized oil, and so forth, are thus further disseminated through the fibrous mass (and into the fibres thereof) composing the sheet. In this way an enhanced degree of water resistance is obtained.

The procedure of the foregoing illustration may be varied in different ways, as for example, a cheaper paper stock may be made by utilizing 3 parts by weight of ground wood 110 to 1 part of sulphite or sulphate pulp. The oxidized waterproofing material may be a blown mixture of paraffin wax containing 10 to 20 per cent of hydrocarbon oil. The employment of the blown hydrocarbon oil may 115 be desirable in operations where the paper is to be printed. In other words, the illustration set forth depicts merely one procedure and since numerous variations are possible, it is to be understood that the invention is not 120 restricted in any manner by the specific character of the illustration.

Paper of suitable thickness produced in this manner, for example, of a thickness between 30 and 40 points, may be employed to 125 make paper discs employed as closures for containers, especially milk bottles, by punching into disc form. These discs, containing any printed emblem or other advertising matter may be made for milk bottle purposes of 130

a diameter such that they will seat tightly on the mouth on the bottle. There is thus obtained a closure for containers, said closure being made from paper carrying oxidized 5 paraffin. Stated in another form, a container closure is produced comprising paper carrying oxidized paraffin wax introduced into the paper from an emulsified condition. As a product there is obtained the paper disc 10 waterproofed with oxidized paraffin, with or without other oxidized hydrocarbons. The features of this disc have been set forth rather fully in the aforesaid patent application Serial No. 107,461, and for further details 15 reference is made to said application.

Larger discs may be punched which can be drawn into the form of a hood cap to be placed about the mouth of the bottle to serve as a cover therefor.

20 In addition to these specific parts of containers, it should be understood that the entire container may be made from paper or pulp containing blown hydrocarbons. Thus, the walls and bottom of a container for milk 25 may be made of board carrying sufficient oxidized wax to render such container tight and water resistant. Boxes for various foods, oyster pails, ice cream containers, and the like, may be produced from paper stock containing the blown wax or such wax with 30 blown petroleum oils.

As pointed out in Serial No. 107,461 it is 35 important in making paper for food products to avoid the introduction of any substances which will possess strong odors and have a contaminating influence on food products such as milk, butter, and the like. Therefore, in preparing paper for such food product containers, I prefer to avoid substances 40 such as blown tars, blown asphalts, and the like, which would be of a contaminating character and which further being dark in color would discolor the paper. Preferably, therefore, I employ oxidized hydrocarbons which 45 are light in color, free or substantially free from odor and which do not impart any objectionable taste to the food material in contact therewith. If oxidation of the paraffin wax is carried to a stage where dark colored 50 resinous substances or strongly odoriferous aldehydes, and the like, result, these when present in paper used in packing foodstuffs may exert a contaminating influence. For such purposes, therefore, I prefer to keep the 55 oxidation within that range where resinous substances substantially are not formed and the physical appearance of the wax which has been subjected to incipient oxidation is only very slightly altered.

60 In the illustration set forth above 4 per cent of the oxidized waxy material is recommended. This is a high proportion for many purposes and 1 or 2 per cent of the blown material may be used advantageously in such 65 cases. On the other hand, for making waxed

paper and using blown wax, I may increase the proportion to produce the desired waxed effect.

Paper which has been made with the aid of the blown wax may, if desired, be superficially waxed, either with the ordinary paraffin wax or with the blown wax, or with any other waxy material or mixture. Hence if the paper disc milk bottle closures formed with the aid of the blown wax require a waxy 70 surfacing for any reason such treatment is 75 not precluded.

It should be understood that I am not precluded from adding unoxidized oils and waxes to the blown wax or blown mixtures 80 of hydrocarbons, when for any reason such admixture is desired, as for example, to cheapen the product.

In Patent No. 1,607,519 to Carleton Ellis, granted November 16, 1926, there is a disclosure of the use of oxy-paraffin in dispersions employed for waterproofing paper. But that companion patent is directed to rosin sized papers containing wax, and more particularly fibrous material produced from 85 pulps containing hydrocellulose. The instant application is particularly directed to the products resulting from the use of oxidized paraffin wax.

What I claim is:— 95

1. Paper carrying oxidized wax.
2. Paper carrying a blown mixture of wax and petroleum oil.
3. Paper containing blown wax in a state of incipient oxidation.

4. Paper containing blown wax free from 100 objectionable resinous substances capable of contaminating foodstuffs.

5. Oxy-paraffined paper.

6. Paper waterproofed with a wax dispersion, a portion at least of the wax content 105 being oxidized paraffin.

7. Paper waterproofed with air blown paraffin wax.

8. Paper carrying oxidized hydrocarbons 110 of substantially non-pigmenting power.

9. Paper carrying blown wax in an amount sufficient to produce a waxed effect in the paper.

10. Paper carrying blown wax softened 115 with an oil.

11. A paper product carrying paraffin wax blown to a state of incipient oxidation.

12. A paper product carrying oxidized 120 paraffin wax and another wax.

13. A paper product carrying a blown mixture of waxes.

14. Paper carrying an oxidized mixture of waxes one of which is paraffin wax, and petroleum oil.

15. A paper product carrying a blown wax and a paper size.

16. Paper carrying oxidized paraffin and a 125 rosin size.

17. A calendered paper product carrying blown wax.

18. A hot calendered paper product carrying oxidized paraffin wax.

19. Paper containing hydrocellulose and carrying oxidized wax.

20. A paper product made from paper containing hydrocellulose and carrying blown paraffin wax.

21. A calendered paper product made from paper containing hydrocellulose and carrying oxidized paraffin and a rosin size.

CARLETON ELLIS.

15

20

25

30

35

40

45

50

55

60